

March 5, 1957

A. MAURIN

2,784,156

METHOD OF AND APPARATUS FOR THE PROTECTION OF COPPER

Filed June 29, 1954



Inventor:  
Alexandre Maurin  
by Robert Henderson  
attorney

1

2,784,156

## METHOD OF AND APPARATUS FOR THE PROTECTION OF COPPER

Alexandre Maurin, Paris, France, assignor to Compagnie de Construction de Gros Materiel Electro Mecanique, Paris, France, a company of France

Application June 29, 1954, Serial No. 440,191

Claims priority, application France August 3, 1953

8 Claims. (Cl. 204—147)

Condenser tubes supplied with sea water, for example those which are installed on board ships and those installed in power stations on land in the vicinity of the sea, are usually made of copper or copper alloys (brass with or without arsenic, to which tin is added, if necessary, and cupro-nickels to which may be added iron and manganese). In spite of the great resistance of copper and its alloys to corrosion by sea water, such corrosion is not negligible in certain cases, and in particular when the water contains an appreciable quantity of organic matter and micro-organisms.

It is an object of the present invention to provide an improved method for preventing corrosion of copper and alloys of copper in contact with salt water, especially in the case of condenser tubes through which sea water is circulated.

During the course of my researches on corrosion in such conditions, I have found that, in order to achieve the desired result, it is desirable to form a homogeneous protecting layer of iron oxide  $Fe_2O_3$  on the surfaces of the copper or the copper alloys, and to maintain this layer on these surfaces by attacking the causes of deterioration of such a layer; furthermore, I have found that there is no corrosion at all when the surface in question is directly covered with the oxide  $Fe_2O_3$ ; that the corrosion is small when there is present an intermediary layer of oxide  $Cu_2O$ , and that, on the other hand, the corrosion is considerable when the surface is coated with cuprous chloride  $CuCl_2$  which is itself covered with a coating of iron oxide  $Fe_3O_4$ ; there is produced by reduction through the agency of bacteria,



the hydrogen sulphide being produced by sulfate-reducing bacteria (e. g. *Sporovibrio desulfuricans*) as explained for example in Herbert Uhlig, Corrosion Handbook, page 469, November 1953, John Wiley & Sons, publishers.

The invention includes the process in accordance with which the salt water, which is destined to come into contact with the surface to be protected, is permanently subjected to an electrolytic action by means of an iron anode, so as to give rise to the formation and transportation of chlorine which plays the part of an oxidising agent and of a bacteria-killing substance, and also ferrate ion  $FeO_4^{2-}$ , which for example is able to be converted to  $Fe_2O_3$  by reduction.

There is an advantage in completing this process by a treatment which enables the formation of a coating of copper oxide, which is insoluble and serves to protect the surface of the copper or copper alloy, the coating being preferably in the form of a brown complex of manganese dioxide  $MnO_2$  and copper oxide  $CuO$ .

To this end, it is recommended to treat the surface in the first place with an aqueous solution of a permanganate, in particular potassium permanganate, for example a solution containing about 0.2 to 0.4 gram of this salt per

2

litre of fresh water. If necessary, the surface to be protected may be first of all cleaned, de-greased and pickled following any one of the known techniques.

In addition, with the object of maintaining the deposit of manganese dioxide on the surface to be protected, it is an advantage to employ a manganese anode, in addition to the iron anode, for the electrolysis of the water which comes into contact with the surface in question; in this way there is formed a manganese ion  $MnO_4^{2-}$  which can be reduced to manganese dioxide.

The reduction of the oxides is mainly effected by means of hydrogen which is given off at the cathode together with sodium hydroxide.

In the case in which the surface of copper or copper alloy is represented by condenser tubes supported by tubular plates which are themselves mounted in a casing made of a ferrous alloy, this casing will preferably be employed as the cathode, since it is then along the walls thereof that sodium hydroxide is produced in the nascent state and makes the water alkaline, by virtue of which the said walls are protected against corrosion. In addition, the concentration of copper chloride on the walls of the tubes is thereby reduced, since such concentration becomes progressively less as the degree of alkalinity of the water increases.

Finally, the invention comprises a protective arrangement which will be illustrated by means of an example of its application to a tubular condenser.

The description which follows below with respect to the attached drawing (which is given by way of example only and not in any sense by way of limitation) will make it quite clear how the invention may be carried into effect; the special features which are brought out, either in the text or in the drawing, being understood to form a part of the said invention.

The single figure represents a diagrammatic illustration of a tubular condenser employing circulation of salt water and provided with an arrangement for protecting it against corrosion.

The condenser comprises a bundle of tubes 1, of copper or copper alloy, held in tubular plates 2, 3. The latter are enclosed in a casing, the end members 4, 5, of which are, for example, made of cast-iron and the cylindrical wall 6, of sheet steel.

In accordance with a special feature of the invention, the tubular plates 2, 3 instead of being directly fixed to the wall 6, are fixed to it through the medium of insulating joints 7, 8, which prevent any direct electrical contact between the copper and the iron.

The casing 4, 5, is supplied with salt water for cooling (for example sea water) through a pipe 9, for example by means of a pump 10, and this water egresses through a pipe 11; the pump 10 draws water from an incoming feed channel 12.

In accordance with the present invention, an iron anode which may be composed of a number of plates 13, is immersed in the channel 12 whilst a second anode 14 made of manganese is preferably located inside the inlet chamber 15 for casing 4, 5. The end members 4, 5 are employed as cathodes, the various electrodes 13, 14, 4, 5, being connected, for example, to a rectifier which has been shown diagrammatically at 16.

The electrolytic protection arrangement which is thus added to the condenser and to its water supply system ensures the formation of ferrate ion  $FeO_4^{2-}$  along plates 13, this oxide being then conveyed by the water circulated by the pump; it also ensures the production at the anodes 13 and 14, of chlorine which effectively destroys bacteria; the reduction of the ferrate ion  $FeO_4^{2-}$  along the surfaces of copper or copper alloys, accompanied by the formation of the oxide  $Fe_2O_3$ , which is deposited there; and finally, the alkalinisation of the water from the

point of its entry into the casing 4, 5, which thereby provides a protection of the ferrous metal whilst at the same time reducing the degree of concentration of copper chloride  $CuCl_2$ .

As has already been stated above, the example which has just been described is solely intended to illustrate the invention and is not to be assumed to have any limiting character.

What I claim is:

1. A process for preventing corrosion by salt water, of the surface of a material containing copper which in operation is in contact with flowing salt water, which comprises continuously passing said flowing salt water before it reaches said surface, through an electrolyzing zone having a cathode and an iron anode therein so as to form an alkaline cathodic product and an iron-containing anodic product in said water in said zone, and continuously passing the whole effluent from said electrolyzing zone including said cathodic and anodic products along said surface.

2. A process for preventing corrosion by salt water, of the surface of a material containing copper which in operation is in contact with flowing salt water, which comprises the initial step of oxidizing said surface to provide a protective film containing copper oxide  $CuO$  thereon, then the step of continuously passing said flowing salt water before it reaches said surface, through an electrolyzing zone having a cathode and an iron anode therein so as to form an alkaline cathodic product and an iron-containing anodic product in said water in said zone, and continuously passing the whole effluent from said electrolyzing zone including said cathodic and anodic products along said surface.

3. A process for preventing corrosion by salt water, of the surface of a material containing copper which in operation is in contact with flowing salt water, which comprises the initial step of contacting an aqueous solution of an alkali metal permanganate with said surface to oxidize the same superficially and to provide a protective film of a brown manganese dioxide-copper oxide complex salt thereon, then the step of continuously passing said flowing salt water before it reaches said surface, through an electrolyzing zone having a cathode, an iron anode and a manganese anode between said iron anode and said surface, so as to form an alkaline cathodic product and an iron- and manganese-containing anodic product in said zone, and passing the whole effluent from said electrolyzing zone including said cathodic and anodic products along said surface.

4. In a heat exchange plant comprising a heat exchange surface made of a material containing copper, the

combination of a salt water receiver, spaced apart from said heat exchange surface; a source of direct electric current; an iron anode in said receiver connected to said source, for producing an anodic product in the salt water in said receiver; piping means for leading said salt water with said anodic product therein from said receiver to said heat exchange surface and passing the same along said surface; and a cathode in said piping means at a point intermediate said iron anode and said heat exchange surface, connected to said source for producing a cathodic product in said salt water containing said anodic product on its way to said heat exchange surface.

5. The combination of claim 4, further comprising a manganese anode, connected to said source, at a point intermediate said iron anode and said heat exchange surface.

6. In a heat exchange plant, the combination of a condenser including a bundle of tubes made of a material containing copper; means comprising an inlet heading

20 secured to but electrically insulated from said bundle of tubes on the inlet side thereof, for leading salt water to the inlet end of said tubes and through said tubes; an iron anode in said means at a point upstream with respect to said inlet heading; a cathode in said inlet heading; and 25 a source of direct electric current between said anode and said cathode.

7. The combination of claim 6, further comprising a manganese anode in said heading.

8. In a heat exchange plant, the combination of a condenser including a bundle of tubes made of a material

30 containing copper; an iron inlet heading and an iron outlet heading for said condenser, secured to but electrically insulated from said condenser; means for feeding salt water to said inlet heading and passing the same through 35 said tubes into and out of said outlet heading; an iron anode in said means at a point upstream with respect to said inlet heading; a manganese anode within said inlet heading, supported and electrically insulated therefrom; a source of direct electric current; means for electrically 40 connecting said iron headings to the negative terminal of said source; and means for electrically connecting said iron anode and manganese anode to the positive terminal of said source.

45 References Cited in the file of this patent

UNITED STATES PATENTS

|           |                         |               |
|-----------|-------------------------|---------------|
| 1,319,508 | Bengough et al. -----   | Oct. 21, 1919 |
| 1,335,209 | von Wurstemberger ----- | Mar. 30, 1920 |
| 2,155,964 | Bowers et al. -----     | Apr. 25, 1939 |